

May 4, 1926.

1,583,198

J. B. STRAUSS

METHOD OF PROTECTING METAL AND METAL STRUCTURES

Filed May 5, 1922



Inventor:  
Joseph B. Strauss  
By Parker & Carter  
Atty.

## UNITED STATES PATENT OFFICE.

JOSEPH B. STRAUSS, OF CHICAGO, ILLINOIS.

## METHOD OF PROTECTING METAL AND METAL STRUCTURES.

Application filed May 5, 1922. Serial No. 558,759.

*To all whom it may concern:*

Be it known that I, JOSEPH B. STRAUSS, a citizen of the United States, residing at Chicago, in the county of Cook and State of Illinois, have invented a certain new and useful Improvement in Methods of Protecting Metal and Metal Structures, of which the following is a specification.

This invention relates to a method of protecting metal and metal structures and consists in providing a new and improved method of this description. Metal structures are subject to deterioration due to the oxidation of the metal. It is customary to apply paint of some kind to prevent this, but this paint lasts only a short time and must therefore be applied at comparatively short intervals and is exceedingly expensive, and if for any reason it is not applied at frequent intervals, the metal structure rapidly deteriorates. The present invention has for its object to provide a method of easily, quickly and cheaply applying a protecting coating to a metal structure either before or after the metal is in position, and which will last for a long period of time and protect the metal from deterioration.

In carrying out this method I first apply to the metal one heavy coat or more of paint completely covering the surface. I then apply an adhesive material, such as glue of some description. Finally I apply a silica coating preferably sprayed in position, as by a current of air. It may for example be applied by means of a cement gun or similar construction, or if desired it may be applied by impacting it either by hand or by mechanism against the surface containing the adhesive and paint. I may, for example, use powdered glass or pebbles or sand for this outer coating, and I may omit the glue surface and employ a paint containing a percentage of glue. This material embeds itself in the glue and paint and completely protects the paint, which in turn protects the metal.

Painting as now done satisfactorily protects the metal as long as the coat of paint remains intact, but when under the action of weather, wind, and rain the paint coat is ruptured or scales off, its protective effect is destroyed. In this new process this is eliminated. The protecting coat may be easily, quickly and cheaply applied and when once properly applied will stay in position and thus completely protect the metal. This coating may be applied either before or after the metal is in position.

For purposes of illustration I have shown a cross-sectional view of a piece of metal showing one form in which the coating is applied. In this drawing there is a piece of metal 1 provided with a coat of paint 2 and an adhesive 3, there being material 4 in a finely divided state embedded in the adhesive. This finely divided material may be any suitable non-oxidizing material such as silica.

I claim:

1. The method of protecting metal and metal structures from deterioration which consists in applying paint and an adhesive to the surface of the metal, and then applying nonoxidizing material in a finely divided state so as to cause it to be held in place by the adhesive to protect the paint.

2. The method of protecting metal and metal structures from deterioration which consists in applying a coat of paint to the metal, then applying an adhesive on the outside of said paint, and then applying non-oxidizing material in a finely divided state while the adhesive is in a plastic condition so as to cause such finely divided material to be embedded in said adhesive to protect said paint.

Signed at Chicago county of Cook and State of Illinois, this 21 day of April 1922.

JOSEPH B. STRAUSS.